

# UNITED STATES PATENT OFFICE.

GEORGE F. POTTLE, OF MEDFORD, MASSACHUSETTS.

## ALLOY OF COPPER, NICKEL, AND LEAD.

SPECIFICATION forming part of Letters Patent No. 390,251, dated October 2, 1888.

Application filed July 2, 1887. Serial No. 243,208. (Specimens.)

*To all whom it may concern:*

Be it known that I, GEORGE F. POTTLE, of Medford, in the county of Middlesex and State of Massachusetts, a citizen of the United States, 5 have invented certain new and useful Improvements in Alloys of Copper, Nickel, and Lead, of which the following is a specification.

My present improvement relates to an improved compound metal or alloy which is particularly adapted to be used to form the facing or bearing-surfaces of journal-boxes and steam or water gates and the sabots of projectiles when these articles are made by first casting the bearing-face in a suitable mold, 15 and afterward uniting or welding with this bearing-face the rest or backing of the article, which is made of a suitable cheap metal, preferably ordinary cast-iron. This latter metal may be caused to unite or weld with the facing metal by flowing it (the backing metal) into a suitable mold in which the facing-piece has already been placed. The capacity which my improved alloy or composition metal has of thus being united or joined with the backing metal in the process of casting constitutes 20 one of its most desirable features.

To form my improved alloy or composition I take six parts, by weight, of commercial copper to one part, by weight, of commercial 25 nickel. These may be melted together in any suitable manner; but I prefer to first melt the nickel in a crucible, and then to add the desired amount of copper, the heat of the molten nickel being sufficient to fuse and unite the

two. To the molten copper and nickel I add 35 one-half a pound of commercial lead, this being added when the mass of copper and nickel has cooled sufficiently not to volatilize the lead.

I do not claim to be the first to form a composition metal in which copper, nickel, and 40 lead enter as ingredients. The novelty of my present invention and its value for the uses hereinbefore set forth lie in the peculiar qualities and advantages found in a metal containing the ingredients in substantially the proportions stated, which composition or combination of ingredients I believe to be new with myself, as well as particularly adapted for the 45 purposes set forth.

While the proportions given above are precisely those which I have found to be adapted 50 to give the best results, I have also discovered that a slight variation in the proportions may be made without affecting the quality of the alloy, as set forth.

I claim—

The herein-described composition or alloy of copper, nickel, and lead, in the proportion of six parts, one part, and one-half a part, by weight, respectively.

In testimony whereof I have hereunto subscribed my name this 30th day of June, A. D. 1887.

GEORGE F. POTTLE.

Witnesses:

J. HENRY TAYLOR,  
E. B. TOMLINSON.